

3,674,499  
SILVER HALIDE PHOTOGRAPHIC SUPER-  
SENSITIZED EMULSION

Keisuke Shiba, Masanao Hinata, Nobuo Tusji, Takushi Miyazaki, and Akira Sato, Kanagawa, Japan, assignors to Fuji Photo Film, Ltd., Nakanuma, Minami Ashigara Machi, Ashigara-Kamigun, Kanagawa, Japan  
No Drawing. Filed May 27, 1970, Ser. No. 41,092  
Claims priority, application Japan, May 27, 1969,

44/41,169

Int. Cl. G03 1/10

U.S. Cl. 96—123

27 Claims

### ABSTRACT OF THE DISCLOSURE

A supersensitizing combination for use in a photographic emulsion comprising (1) a sensitizing dye having the general formula

General Formula I



wherein the symbols R, R<sub>1</sub>, R<sub>2</sub>, R<sub>3</sub>, R<sub>4</sub>, R<sub>5</sub>, X, Y, Y<sub>1</sub>, Q, n<sub>1</sub>, n<sub>2</sub>, n<sub>3</sub>, n<sub>4</sub> and m are described hereinafter, and (2) a condensate of formalin with a halogenated polyhydroxy benzene or a halogenated cresol, is disclosed.

### BACKGROUND OF THE INVENTION

#### (1) Field of the invention

This invention relates to a silver halide photographic emulsion. More particularly, it is concerned with a so-called supersensitized silver halide photographic emulsion.

#### (2) Description of the prior art

It is well known that the addition of a sensitizing dye to a silver halide emulsion in making a photographic emulsion optically sensitizes the silver halide emulsion and enlarges its sensitive spectral region.

When a sensitizing dye and a compound which does not sensitize the same spectral region as the sensitizing dye are added to a silver halide emulsion, at least a part of the spectral region which the sensitizing dye sensitizes sometimes is sensitized more strongly than when the sensitizing dye alone is added in the same amount to the silver halide emulsion. In this case, the silver halide emulsion may be considered to be supersensitized. Such compounds which do not sensitize the same spectral region as sensitizing dyes are called supersensitizers.

### SUMMARY OF THE INVENTION

It has been found that supersensitization is obtained by adding to a silver halide photographic emulsion a sensitizing dye represented by the following general Formula I in combination with a "halogenated polyhydroxybenzene-formalin condensate" or a "halogenated cresol-formalin condensate." The term "halogenated polyhydroxybenzene" means a halogen-substituted benzene having from one to three hydroxyl groups in the benzene nucleus. Further, the term "halogenated polyhydroxybenzene-formalin condensate" or "halogenated cresol-formalin condensate" will hereinafter be referred to as "formalin condensate."

General Formula I



In this general formula, R<sub>1</sub> and R<sub>2</sub> are each respectively alkyl groups, such as methyl, ethyl, and propyl groups; substituted alkyl groups such as  $\beta$ -hydroxyethyl,  $\beta$ -acetoxymethyl,  $\gamma$ -acetoxymethyl,  $\beta$ -sulfatoethyl ( $-\text{C}_2\text{H}_4\text{OSO}_3\text{H}$ ),  $\gamma$ -sulfatopropyl ( $-\text{C}_3\text{H}_6\text{OSO}_3\text{H}$ ), carboxymethyl,  $\beta$ -carboxymethyl, 2-(2-carboxyethoxy)ethyl,  $\beta$ -ulfoethyl,  $\gamma$ -sulfopropyl,  $\delta$ -sulfovutyl, 2-hydroxy 1-sulfopropyl, 2-(3-sulfopropoxy)ethyl, 2-acetoxymethyl, 3-methoxy-2-(3-sulfopropoxy)-propyl, 2-2-(3-sulfopropoxy)ethoxyethyl, and 2-hydroxy-3-(3'-sulfopropoxy)-propyl; allyl groups; aryl groups; substituted aryl groups, such as  $\rho$ -carboxyphenyl,  $\rho$ -sulfophenyl; and aralkyl groups; R is an alkyl group, a substituted alkyl group, such as a hydroxyalkyl group, a carboxyalkyl group, a sulfoalkyl group, and the like, or an allyl group; R<sub>3</sub> is a hydrogen atom, an alkyl group or an aryl group; R<sub>4</sub> is a hydrogen atom, an alkyl group, such as methyl or ethyl group; or a substituted alkyl group such as a  $\beta$ -ethoxyethyl or a  $\beta$ -( $\gamma$ -sulfopropoxy)-ethyl

group, and when n<sub>4</sub> is 0, R<sub>4</sub> may be connected through the methine chain with a nitrogen atom in a heterocyclic ring completed by Y<sub>1</sub>; R<sub>5</sub> is a hydrogen atom, an alkoxy group, such as a methoxy or an ethoxy group; or a substituted alkoxy group, such as a  $\gamma$ -sulfopropoxy or a  $\beta$ -methoxyethoxy group; n<sub>1</sub>, n<sub>3</sub> and n<sub>4</sub> are respectively 0 or 1, n<sub>2</sub> is 0, 1 or 2, Q is an oxygen atom, a sulfur atom or  $-\text{N}(\text{---R}_6)$ , wherein R<sub>6</sub> is an alkyl group such as a methyl or an ethyl group; Y and Y<sub>1</sub> each represent, for example, the nonmetallic atoms necessary to complete a heterocyclic nucleus of the thiazole series (for example, thiazole, 4-methylthiazole, 4-phenylthiazole, 5-methylthiazole, 5-phenylthiazole, 4,5-dimethylthiazole, 4,5-diphenylthiazole, or 4-(2-thienyl)thiazole), of the benzthiazole series (for example, benzthiazole, 4-chlorobenzthiazole, 5-chlorobenzthiazole, 6-chlorobenzthiazole, 7-chlorobenzthiazole, 4-methylbenzthiazole, 5-methylbenzthiazole, 6-methylbenzthiazole, 5-bromobenzthiazole, 6-bromobenzthiazole, 4-phenylbenzthiazole, 5-phenylbenzthiazole, 4-methoxybenzthiazole, 5-methoxybenzthiazole, 6-methoxybenzthiazole, 5-iodobenzthiazole, 6-iodobenzthiazole, 4-ethoxybenzthiazole, 5-ethoxybenzthiazole, tetrahydrobenzthiazole, 5,6-dimethoxybenzthiazole, 5,6-dioxymethylenebenzthiazole, 5-hydroxybenzthiazole, or 6-hydroxybenzthiazole), of the naphthothiazole series (for example,  $\alpha$ -naphthothiazole,  $\beta$ -naphthothiazole, 8-methoxy- $\alpha$ -naphthothiazole or 7-methoxy- $\alpha$ -naphthothiazole), of the benzoxazole series (for example, benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 5-ethoxybenzoxazole, 6-methoxybenzoxazole, 5-hydroxybenzoxazole or 6-hydroxybenzoxazole), of the naphthoxazole series (for example,  $\alpha$ -naphthoxazole or  $\beta$ -naphthoxazole), of the selenazole series (for example, 4-methylselenazole or 4-phenylselenazole), of the benzoselenazole series (for example, benzoselenazole, 5-chlorobenzoselenazole, 5-methoxybenzoselenazole, 5-hydroxybenzoselenazole, or tetrahydrobenzoselenazole), of the naphthoselenazole series (for example,  $\alpha$ -naphthoselenazole or  $\beta$ -naphthoselenazole), of the thiazoline series (for

example, thiazoline or 4-methylthiazoline), of the 2-quinoline series (for example, quinoline, 3-methylquinoline, 5-methylquinoline, 7-methylquinoline, 8-methylquinoline, 6-chloroquinoline, 8 - chloroquinoline, 6-methoxyquinoline, 6-ethoxyquinoline, 6-hydroxyquinoline or 8-hydroxyquinoline), of the 4-quinoline series (for example, quinoline, 6-methoxyquinoline, 7-methylquinoline or 8-methylquinoline), of the 1-isoquinoline series (for example, isoquinoline itself), of the benzimidazole series (for example, 1,3-diethylbenzimidazole or 1-ethyl-3-phenylbenzimidazole), of the 3,3-dialkyldolene series (for example, 3,3-dimethylindolene, 3,3, 5-tri-methylindolene, or 3,3,7-trimethylindolene), or of the pyridine series (for example, pyridine or 5-methylpyridine), X is an anion used in the sensitizing dye, such as a halogen ion, perchlorate, thiocyanate, p-toluene-sulfonate, benzenesulfonate, ethylsulfate, methylsulfate, and the like, and m is 1 or 2, m being 1 where an intramolecular salt is formed.

The halogenated polyhydroxybenzene used in the invention is represented by the following general formula



wherein n ranges from 1 to 3, n' ranges from 1 to 3 wherein simultaneously n and n' cannot both be 3, wherein X<sub>1</sub> is a chlorine or bromine atom.

Examples of the compounds represented by the above mentioned general formula are o-chlorophenol, m-chlorophenol, p-chlorophenol, o-bromophenol, m-bromophenol, p-bromophenol, 2,4-dichlorophenol, 2,6-dichlorophenol, 2, 5-dichlorophenol, 2,4-dibromophenol, 2,5-dibromophenol, 2 - chlorohydroquinone, 4-chlororesorcinol, 4-chlorocatechol, 2-bromohydroquinone, 4-bromoresorcinol, 4-bromo-resorcinol, 4-bromocatechol, and 2,4,5-trichlorophenol.

The halogenated cresol used in the invention is represented by the following general formula



wherein X<sub>1</sub> is a chlorine or bromine atom.

Examples of compounds represented by the above mentioned general formula are 6-chloro-m-cresol, p-chloro-o-cresol and p-chloro-m-cresol.

Synthesis of the condensate of the halogenated polyhydroxybenzene and formalin can be carried out according to the conventional synthesis method for a phenol-formaldehyde resin of the novolak type. The general synthesis method is as follows: The halogenated polyhydroxybenzene is dissolved or dispersed in water, to which a mineral acid, such as concentrated hydrochloric acid or sulfuric acid, and 37% formalin (aqueous solution of formaldehyde) are added, and the mixture is heated at 100° C. for from 30 minutes to 1 hour with agitation. The reaction can be carried out under a pressure in an autoclave. After the reaction, the product is poured in cold water and the resultant precipitate is purified.

Another example is as follows: 400 parts of o-chlorophenol is dispersed in 1,000 parts of water with vigorous agitation, to which 25 parts of 35% hydrochloric acid and 250 parts of 37% formalin are then added. Then, the reaction mixture is heated at 100° C. with stirring and held for 30 minutes. 20 parts of concentrated hydrochloric acid is added additionally and the reaction is further continued for another 30 minutes. 20 parts of concentrated hydrochloric acid is then added and stirred to give a white turbidity. After about 1 hour and 30 minutes, the stirring is stopped and the mixture is transferred into 3,000 parts of cold water with agitation. The resulting precipitate is filtered, not dried, re-dissolved in 500 parts of methanol and precipitated again with cold water. Then, the precipitate is filtered and dried to obtain the desired product.

Other formalin condensates can be obtained readily in a similar manner or in the somewhat varied manner. However, the preparation of the formalin condensate used in the invention is not limited to the above described method, but can be carried out using other suitable methods.

The formalin condensate used in the invention has a condensation unit (degree of polymerization) of from 2 to 10 similar to the conventional novolak resins. For the purposes of the invention, a degree of polymerization of from 2 to 10, preferably from 2 to 5, as well as a molecular weight of from 250 to 750 is desired.

Examples of the sensitizing dye of the invention represented by the foregoing general Formula I are given in the following without limiting the invention.



I-3



I-4



I-5



I-6



I-7



I-8



I-9





I-17



I-18



The sensitizing dye used in the invention may be synthesized in known manner per se such as the method as disclosed in U.S. Pat. 2,947,680. Several synthetic examples are as follows:

#### SYNTHETIC EXAMPLE 1

##### Synthesis of I-3

4.2 g. of 3-ethyl-5-[3-ethyl-naphtho[2,1-d]thiazol-5-ylidene]-1-phenylethylidene-rhodanine and 2.0 g. of methyl p-toluenesulfonate are reacted by heating at 140° C. for 2 hours. To the reaction product is added a reaction product obtained by reacting 2 g. of 3-ethyl-2-acetyl-methylenebenzothiazoline and 2.3 g. of  $\beta$ -methoxyethyl p-toluene-sulfonate by heating at 145° C. for 3 hours, and reacted in 80 ml. of ethanol and 4 ml. of triethylamine by heating and refluxing on a warm water bath for 2 hours. After the reaction, the reaction solution is concentrated and added to an aqueous solution of sodium bromide. The precipitated crystal is washed with water, dried, treated with ethyl acetate to remove the soluble materials and then recrystallized from ethanol to obtain 1.2 g. of I-3 melting at 212° C.

$\lambda_{\text{max}}^{\text{MeOH}}$  673 m $\mu$

#### SYNTHETIC EXAMPLE 2

##### Synthesis of I-5

5 g. of 3-aryl-5-[(1-ethyl-4-quinolinidene)-ethylidene]rhodanine and 4 g. of methyl p-toluenesulfonate are reacted by heating at 110° C. for 1 hour. 3 g. of 3-ethyl-2-( $\gamma$ -ethoxypropyl)benzothiazolium p-toluene-sulfonate is added to the reaction product and reacted in 200 ml. of ethanol and 3 ml. of triethylamine by heating on a warm water bath for 1 hour. During the reaction, crystals are deposited and are filtered subsequently. The resulting crystal is recrystallized from methanol to thus obtain 4 g. of I-5 melting at 270° C.

$\lambda_{\text{max}}^{\text{MeOH}}$  685 m $\mu$

#### SYNTHETIC EXAMPLE 3

##### Synthesis of I-4

I-4 is obtained in a similar manner to the dye I-5. M.P. 256° C.

$\lambda_{\text{max}}^{\text{MeOH}}$  685 m $\mu$

The coexistence of the formaline condensate used in the invention with the sensitizing dye represented by the general Formula I in a silver halide emulsion results in the supersensitizing action, and, simultaneously, reduces fog markedly in comparison with a case where only a sensitiz-

ing dye is incorporated in an emulsion. Some of the sensitizing dyes represented by the general Formula I, incorporated in a photographic material, cause sensitivity lowering on storage, but this disadvantage can favorably be overcome by the incorporation of the formalin condensate of the invention in combination.

The sensitizing dye of the invention is ordinarily used in a silver halide emulsion at a concentration of from 0.002 to 0.2 g./silver halide g. mol and the formalin condensate is used at a concentration of from 0.1 to 5.0 g./silver halide g. mol, the concentration ratio of the sensitizing dye and formalin condensate preferably ranging from 1:5 to 1:500. Addition of the sensitizing dye can be carried out using methods known to those skilled in the art. For example, the formalin condensate can be added to a silver halide emulsion in the form of a solution in an organic solvent such as methanol or ethanol. The sensitizing dye and formalin condensate are preferably added to an emulsion before the application of the emulsion. The order of addition to the emulsion is not limited particularly. Any of the sensitizing dyes and the formalin condensate can be added firstly or the both can be added in admixture. Furthermore, they can be added to an emulsion after water washing and during ageing.

In the invention, a conventional gelatino-silver halide emulsion is used but other resinous materials and cellulose derivatives, compatible with photographic materials, can be used of course. Silver halides such as silver chloride, silver bromide, silver iodobromide, silver chlorobromide or silver chloriodobromide, can be used for the emulsion of the invention.

The emulsion of the invention also can contain conventional additives such as chemical sensitizers, fog inhibitors, stabilizers, hardeners, coating aids, plasticizers, development accelerators, color tone regulators, whitening agents and couplers. The emulsion can be applied in the conventional manner to a suitable support such as a glass sheet, a cellulose derivative film, a synthetic resin film or a baryta paper.

The following examples are to illustrate the invention further without limiting it.

#### EXAMPLES

(1) The sensitizing dye represented by the general Formula I and (2) the sensitizing dye represented by the general Formula I and a formalin condensate were respectively added to different portions of the same batch of a silver halide emulsion and coated onto cellulose acetate bases followed by drying, exposing through a Fuji K Filter-7 (made by Fuji Photo Film Co.) transmitting wavelengths longer than 590 millimicrons and developing. The results

obtained are shown in Table 1 below in which the sensitivity means the value of the exposure quantity necessary for giving a fog and optical density of 0.1, based on a sensitivity of 100 in the case of incorporating the sensitizing dye only. There was no or little sensitization in the case of incorporating the formalin condensate only (not shown). In each example for comparison the same batch of the emulsion is used, but in other examples several different emulsions are used. In Examples 1 to 8, the same batch of the silver chlorobromide (Br 40 mol percent, Cl 10



60 mol percent) was used, in Examples 9 to 16 the same batch of silver chlorobromide (Br 50 mol percent, Cl 50 mol percent) was used and in Examples 17 to 19 the same batch of silver iodobromide (I-5 mol percent, Br 95 mol percent) was used. The development is carried out at 20° C. for 2 minutes with a developer as shown in Table 2 for Examples 1 to 16 and at 20° C. for 4 minutes with a developer as shown in Table 3 for Examples 17 to 19.

TABLE I

| Additives (mg./silver halide g. mol)                                     | Sensitivity | Fog  |
|--------------------------------------------------------------------------|-------------|------|
| (a) I-7 (69.0)                                                           | 100         | 0.19 |
| (b) I-7 (69.0) plus o-chlorophenol-formaldehyde condensate (1,460)       | 315         | 0.08 |
| (c) I-7 (69.0) plus p-chlorophenol-formaldehyde condensate (1,460)       | 575         | 0.07 |
| (d) I-7 (69.0) plus p-bromophenol-formaldehyde condensate (1,460)        | 398         | 0.08 |
| (e) I-7 (69.0) plus 2, 4-dichlorophenol-formaldehyde condensate (1,460)  | 251         | 0.08 |
| (f) I-7 (69.0) plus 2-chlorohydroquinone-formaldehyde condensate (1,460) | 225         | 0.10 |
| (g) I-7 (69.0) plus 4-chlororesorcinol-formaldehyde condensate (1,460)   | 280         | 0.10 |
| (h) I-7 (69.0) plus 6-chloro-m-cresol-formaldehyde condensate (1,460)    | 225         | 0.08 |
| 1. (i) I-1 (53.5)                                                        | 100         | 0.09 |
| (j) I-1 (53.5) plus p-chlorophenol-formaldehyde condensate (2,920)       | 178         | 0.05 |
| 2. (k) I-2 (78.5)                                                        | 100         | 0.06 |
| (l) I-2 (78.5) plus p-chlorophenol-formaldehyde condensate (2,920)       | 145         | 0.06 |
| 3. (m) I-3 (76.3)                                                        | 100         | 0.06 |
| (n) I-3 (76.3) plus p-chlorophenol-formaldehyde condensate (2,920)       | 365         | 0.05 |
| 4. (o) I-4 (55.7)                                                        | 100         | 0.16 |
| (p) I-4 (55.7) plus p-chlorophenol-formaldehyde condensate (2,920)       | 478         | 0.05 |
| 5. (q) I-5 (71.7)                                                        | 100         | 0.17 |
| (r) I-5 (71.7) plus p-chlorophenol-formaldehyde condensate (2,920)       | 615         | 0.05 |
| 6. (s) I-6 (71.5)                                                        | 100         | 0.16 |
| (t) I-6 (71.5) plus p-chlorophenol-formaldehyde condensate (2,920)       | 315         | 0.05 |
| 7. (u) I-7 (69.0)                                                        | 100         | 0.19 |
| (v) I-7 (69.0) plus p-chlorophenol-formaldehyde condensate (2,920)       | 708         | 0.08 |
| 8. (w) I-8 (68.6)                                                        | 100         | 0.13 |
| (x) I-8 (68.6) plus p-bromophenol-formaldehyde condensate (1,460)        | 210         | 0.09 |
| 9. (y) I-9 (69.7)                                                        | 100         | 0.07 |
| (z) I-9 (69.7) plus p-bromophenol-formaldehyde condensate (1,460)        | 250         | 0.07 |
| 10. (aa) I-10 (57.1)                                                     | 100         | 0.30 |
| (bb) I-10 (57.1) plus p-bromophenol-formaldehyde condensate (1,460)      | 603         | 0.06 |
| 11. (cc) I-11 (55.1)                                                     | 100         | 0.07 |
| (dd) I-11 (55.1) plus p-bromophenol-formaldehyde condensate (1,460)      | 120         | 0.07 |
| 12. (ee) I-12 (66.5)                                                     | 100         | 0.08 |
| (ff) I-12 (66.5) plus p-bromophenol-formaldehyde condensate (1,460)      | 140         | 0.08 |
| 13. (gg) I-13 (69.3)                                                     | 100         | 0.08 |
| (hh) I-13 (69.3) plus p-bromophenol-formaldehyde condensate (1,460)      | 190         | 0.08 |
| 14. (ii) I-14 (64.3)                                                     | 100         | 0.08 |
| (jj) I-14 (64.3) plus p-bromophenol-formaldehyde condensate (1,460)      | 398         | 0.06 |
| 15. (kk) I-15 (73.9)                                                     | 100         | 0.09 |
| (ll) I-15 (73.9) plus p-bromophenol-formaldehyde condensate (1,460)      | 178         | 0.07 |
| 16. (mm) I-16 (60.3)                                                     | 100         | 0.09 |
| (nn) I-16 (60.3) plus o-chlorophenol-formaldehyde condensate (2,920)     | 310         | 0.06 |
| 17. (oo) I-17 (77.5)                                                     | 100         | 0.25 |
| (pp) I-17 (77.5) plus o-chlorophenol-formaldehyde condensate (2,920)     | 251         | 0.07 |
| 18. (qq) I-18 (69.4)                                                     | 100         | 0.19 |
| (rr) I-18 (69.4) plus o-chlorophenol-formaldehyde condensate (2,920)     | 190         | 0.06 |

TABLE 2

|                                    | G.   | 65 |
|------------------------------------|------|----|
| N-methyl-p-aminophenosulfate ----- | 3.1  |    |
| Sodium sulfite -----               | 45   |    |
| Hydroquinone -----                 | 12   |    |
| Sodium carbonate (anhydrous) ----- | 67.5 |    |
| Potassium bromide -----            | 1.9  | 70 |
| Water to 1000 ml.                  |      |    |

TABLE 3

|                              | G.    |
|------------------------------|-------|
| N-methyl-p-aminophenosulfate | 2.2   |
| Sodium sulfite               | 96 75 |

|                   |     |
|-------------------|-----|
| Hydroquinone      | 8.8 |
| Sodium carbonate  | 48  |
| Potassium bromide | 5   |
| Water to 1000 ml. |     |

5

**What is claimed is:**

## 1. A silver halide photographic emulsion containing the combination of

- (1) at least one sensitizing dye having the following general formula



wherein Y and  $Y_1$  each represents the non-metallic atoms necessary to complete a heterocyclic nucleus selected from the group consisting of the thiazole series, of the benzthiazole series, of the naphtho-thiazole series, of the oxazole series, of the benzo-oxazole series, of the naphtho-oxazole series, of the thiazo-line series, of the 2-quinoline series, of the 4-quinoline series of the benzimidazole series, of the 3,3-di-

alkylindolenine series, and of the pyridine series; wherein  $R_1$  and  $R_2$  each is selected from the group consisting of an alkyl group and, a hydroxy-, acetoxy, sulfato-, carboxy-, carboxyalkoxy-, sulfo-, hydroxy-sulfo-, sulfoalkoxy-, alkoxy-sulfoalkoxy-, sulfoalkoxy-alkoxy-, or hydroxy-sulfoalkoxy-substituted aryl group or aralkyl group; wherein  $R$  is selected from the group consisting of an alkyl group, a hydroxy-, carboxy-, or sulfo-substituted alkyl group, and an allyl group; wherein  $R_4$  is selected from the group consisting of a hydrogen atom, an alkyl group and, a sulfoalkoxy-, or alkoxy-substituted alkyl group.

and, when  $n_4$  is 0,  $R_4$  may be connected through the methine chain with a nitrogen atom in the heterocyclic nucleus completed by  $Y_1$ ; wherein  $R_5$  is selected from the group consisting of a hydrogen atom, an alkoxy group and a sulfo-, or alkoxy-substituted alkoxy group; wherein  $n_1$ ,  $n_3$  and  $n_4$  each is 0 or 1; wherein  $n_2$  is 0, 1 or 2; wherein  $Q$  is selected from the group consisting of an oxygen atom, a sulfur atom, and a  $=N-R_6$  group, wherein  $R_6$  is an alkyl group,  $X$  is a negatively charged anion, and wherein  $m$  is 1 or 2, and wherein  $m$  is 1 an intramolecular salt is formed; and

- (2) at least one condensate of formaldehyde with a member selected from the group consisting of a halogenated polyhydroxybenzene having the following general Formula II



and a halogenated cresol having the following general Formula III



wherein  $n$  is 1, 2 or 3; wherein  $n'$  is 1, 2 or 3 and wherein  $n$  and  $n'$  are not simultaneously 3, and wherein  $X_1$  is selected from the group consisting of a chlorine atom and a bromine atom, are incorporated in combination.

2. The emulsion of claim 1, wherein the sensitizing dye is a compound selected from the group consisting of



and



3. The emulsion of claim 1, wherein said halogenated polyhydroxybenzene is selected from the group consisting of o-chlorophenol, m-chlorophenol, p-chlorophenol, o-bromophenol, m-bromophenol, p-bromophenol, 2,4-dichlorophenol, 2,6-dichlorophenol, 2,5-dichlorophenol, 2,4-dibromophenol, 2,5-dibromophenol, 2-chlorohydroquinone, 4-chlororesorcinol, 4-chlorocatechol, 2-bromo-hydroquinone, 4-bromoresorcinol, 4-bromocatechol, and 2,4,5-trichlorophenol.

4. The emulsion of claim 1, wherein said halogenated cresol is selected from the group consisting of 6-chloro-m-cresol, p-chloro-o-cresol, and p-chloro-m-cresol.

5. The emulsion of claim 1, wherein said condensate has a degree of polymerization of 2 to 10.

6. The emulsion of claim 1, wherein the concentration of said sensitizing dye ranges from 0.002 to 0.2 gram per gram mole of silver halide.

7. The emulsion of claim 1 wherein the concentration of said formalin condensate ranges from 1 to 5.0 grams per gram mole of silver halide.

8. The emulsion of claim 1, wherein the weight ratio of the concentration of the sensitizing dye to the formalin condensate ranges from 1:5 to 1:500.

9. The emulsion of claim 1, wherein the combination of the sensitizing dye with the formalin condensation is selected from the group consisting of o-chlorophenol-formaldehyde condensate, p-chlorophenol-formaldehyde condensate, p-bromophenol-formaldehyde condensate, 2,4-dichlorophenol-formaldehyde condensate, 2-chlorohydroquinone-formaldehyde condensate, 4-chlororesorcinol-formaldehyde condensate and 6-chloro-m-cresol-formaldehyde condensate, wherein the sensitizing dye is



10. The emulsion of claim 1, wherein the combination of the sensitizing dye with the formalin condensate is:



75 and p-chlorophenol-formaldehyde condensate.

15

11. The emulsion of claim 1, wherein the combination of the sensitizing dye with the formalin condensate is:



and p-chlorophenol-formaldehyde condensate.

12. The emulsion of claim 1, wherein the combination of the sensitizing dye with the formalin condensate is:



and p-chlorophenol-formaldehyde condensate.

13. The emulsion of claim 1, wherein the combination of the sensitizing dye with the formalin condensate is:



and p-chlorophenol-formaldehyde condensate.

14. The emulsion of claim 1, wherein the combination of the sensitizing dye with the formalin condensate is:



and p-chlorophenol-formaldehyde condensate.

15. The emulsion of claim 1, wherein the combination of the sensitizing dye with the formalin condensate is:



and p-chlorophenol-formaldehyde condensate.

16

16. The emulsion of claim 1, wherein the combination of the sensitizing dye with the formalin condensate is:



and p-bromophenol-formaldehyde condensate.

17. The emulsion of claim 1, wherein the combination of the sensitizing dye with the formalin condensate is:



and p-bromophenol-formaldehyde condensate.

18. The emulsion of claim 1, wherein the combination of the sensitizing dye with the formalin condensate is:



and p-bromophenol-formaldehyde condensate, o

19. The emulsion of claim 1, wherein the combination of the sensitizing dye with the formalin condensate is:



and p-bromophenol-formaldehyde condensate.

20. The emulsion of claim 1, wherein the combination of the sensitizing dye with the formalin condensate is:



and p-bromophenol-formaldehyde condensate.

21. The emulsion of claim 1, wherein the combination of the sensitizing dye with the formalin condensate is:



and p-bromophenol-formaldehyde condensate.

17

22. The combination of claim 1, wherein the combination of the sensitizing dye with the formalin condensate is:



5

I-

and p-bromophenol-formaldehyde condensate.

23. The emulsion of claim 1, wherein the combination

18

and p-bromophenol-formaldehyde condensate.

24. The emulsion of claim 1, wherein the combination of the sensitizing dye with the formalin condensate is:



10

I-

and o-chlorophenol-formaldehyde condensate.

25. The emulsion of claim 1, wherein the combination of the sensitizing dye with the formalin condensate is:



of the sensitizing dye with the formalin condensate is:



40 and o-chlorophenol-formaldehyde condensate.

26. The emulsion of claim 1, wherein the combination of the sensitizing dye with the formalin condensate is:



and o-chlorophenol-formaldehyde condensate.

27. A photographic light-sensitive element comprising a support having thereon at least one layer containing the silver halide emulsion of claim 1.

#### References Cited

##### UNITED STATES PATENTS

2,961,318 11/1960 Jones ----- 96—123  
3,342,606 9/1967 Silver ----- 96—114

##### FOREIGN PATENTS

434,937 2/1968 Japan ----- 96—123

J. TRAVIS BROWN, Primary Examiner

U.S. Cl. X.R.

96—127, 139, 140